

# United States Patent

[19]

Yamakawa et al.

[11] 3,873,379

[45] Mar. 25, 1975

[54] **METHOD OF PRODUCING RARE EARTH-COBALT PERMANENT MAGNET USING SPECIAL COOLING RATES**

[75] Inventors: **Kazuo Yamakawa**, Tokyo; **Tohru Oka**, Kumagaya; **Masaaki Tokunaga**, Kumagaya; **Takeshi Mizuhara**, Kumagaya; **Chitoshi Hagi**, Kumagaya, all of Japan

[73] Assignee: **Hitachi Metals, Ltd.**, Tokyo, Japan

[22] Filed: **July 10, 1973**

[21] Appl. No.: **377,919**

[30] **Foreign Application Priority Data**

July 12, 1973 Japan ..... 47-69106

[52] **U.S. Cl.** ..... **148/103**, 148/31.57, 148/105

[51] **Int. Cl.** ..... **H01f 1/02**

[58] **Field of Search** ..... 148/103, 105, 108, 101, 148/31.57

[56] **References Cited**

UNITED STATES PATENTS

1,752,490 4/1930 Karcher ..... 148/112  
3,663,317 5/1972 Westendorf et al. ..... 148/103

3,682,714 8/1972 Martin ..... 148/31.57  
3,684,593 8/1972 Benz et al. ..... 148/103  
3,755,007 8/1973 Benz et al. ..... 148/101  
3,790,414 2/1974 Tawara et al. ..... 148/31.57

OTHER PUBLICATIONS

Buschow, K. et al., *Perm. Mag. Mt'l's of Rare Earth Cobalt Compounds*, in *Zeit, fur Ang. Physik*, 26, 1969, pp. 157-160.

*Primary Examiner*—Walter R. Satterfield  
*Attorney, Agent, or Firm*—Stewart and Kolasch, Ltd.

[57] **ABSTRACT**

A method of producing a rare earth-cobalt permanent magnet having high coercive force wherein powdery alloy containing rare earth elements and cobalt as principal component is compacted in magnetic field, the resulting green body is sintered at the temperature between 1,000° to 1,200°C, the sintered body is cooled from the above sintering temperature to quenching temperature in the range of 875°±50°C at a rate of 7°C/min. or slower rate, and then further cooled successively from the quenching temperatures to room temperature at a rate of 20°C/min. or faster rate.

**6 Claims, 3 Drawing Figures**

PATENTED MAR 25 1975

3,873,379

FIG. 1



FIG. 2



FIG. 3



**METHOD OF PRODUCING RARE EARTH-COBALT  
PERMANENT MAGNET USING SPECIAL  
COOLING RATES**

**BACKGROUND OF THE INVENTION**

**1. Field of the Invention**

The present invention relates to a permanent magnet consisting of rare earth elements and cobalt.

**2. Description of Prior Art**

Compared with an Alnico type permanent magnet and a ferrite type permanent magnet, a permanent magnet consisting of rare earth elements and cobalt has very high magnetic energy product. Therefore, a rare earth-cobalt permanent magnet has recently been developed in various institutions and factories all over the world.

Rare earth elements for the rare earth-cobalt permanent magnet of the present invention are selected from lanthanide series having atomic number 57 to 71, yttrium and scandium according to the required magnetic properties of the magnet.

While, the magnetic properties of the rare earth-cobalt permanent magnet depend largely upon the preparation process thereof. At present, the following method consisting of the following steps is often used.

i. A step wherein rare earth elements and cobalt are melted together so that a final product, namely alloy having desired composition may be obtained.

In this case, the final product shows the best magnetic properties, when the alloy is the mixture of intermetallic compounds as  $Co_5R$  (R: rare earth elements) and Co-R intermetallic compounds containing richer rare earth elements than  $Co_5R$  does.

The above mentioned alloy contains 55-70 percent by weight of Co and 30-45 percent by weight of rare earth elements. The alloy can contain slight amount of impurities and part of Co thereof can be replaced by Fe or Cu.

ii. A step wherein resulting alloy is ground mechanically to powder whose mesh is few mm in non-oxidative atmosphere.

iii. A step wherein the resulting powdery alloy is compressed by a press under high pressure to obtain green body of adequate shape. In the above molding process, it is useful for the improvement in the magnetic properties of the magnet to give the green body magnetic anisotropy by applying external magnetic field in predetermined direction.

iv. A step wherein the green body is sintered at the temperature between 1,000° to 1,200°C.

v. An additional aging step proposed by Japanese laid patent publication No. 5604/1971 (See U.S. patent application Ser. No. 86,288 and 33,315) wherein the sintered green body is heated to about 900°C and kept at that temperature after sintering to improve further the magnetic properties of a magnet as a final product.

In general, it is preferable that a permanent magnet has as high coercive force, residual induction and energy product as possible. It is well known that these magnetic properties depend largely upon preparation process thereof, above all on heat treatment process.

Therefore, the object of the present invention is to provide a method of producing a rare earth-cobalt permanent magnet having excellent magnetic properties without using aging process.

**SUMMARY OF THE INVENTION**

The present invention relates to a process wherein powdery alloy consisting of rare earth elements and cobalt is molded in magnetic field, the resulting green body is sintered at the temperature between 1,000° to 1,200°C, the sintered body is gradually cooled to the quenching temperature in the range of  $875^\circ \pm 50^\circ C$  at a rate of  $7^\circ C/min.$  or slower rate, and then the sintered body thus cooled is quickly cooled again from the quenching temperature to room temperature at a rate of  $20^\circ C/min.$  or faster rate.

**BRIEF DESCRIPTION OF THE DRAWINGS**

15 FIG. 1 shows the influence of the quenching temperature on the intrinsic coercive force  $H_c$  of cobalt-samarium alloy permanent magnet.

20 FIG. 2 shows the influence of the cooling rate from the sintering temperatures to the quenching temperatures on the intrinsic coercive force  $H_c$  of cobalt-samarium alloy permanent magnet.

25 FIG. 3 shows the influence of the cooling rate from the sintering temperatures to room temperature on the intrinsic coercive force  $H_c$  of cobalt-samarium alloy permanent magnet.

**DETAILED DESCRIPTION OF THE INVENTION**

**EXAMPLE 1**

Powdery alloy whose composition was Sm-57.8-%Co was added to powdery alloy whose composition was Sm-66.2%Co to obtain mixed powdery alloy whose composition was Sm-63.8%Co. The resulting 30 mixed powdery alloy was ground by a vibration mill for 50 minutes to fine powder. The obtained fine powder was molded by compression in a mold under the pressure of  $10 \text{ tons/cm}^2$  in magnetic field of  $8 \text{ KOe}$ . The green body which was in the shape of a rod about 5 mm long and about 10 mm in diameter was sintered 35  $1,140^\circ C$  for 1 hour in an inert gas atmosphere. After the sintering was completed, the sintered body was cooled in a furnace from the sintering temperature to the quenching temperature of  $900^\circ C$  at a rate of  $6^\circ C/min.$  Then the sintered body was immediately and quickly cooled to room temperature by blasting it with argon gas at a rate of  $200^\circ C/min.$  The magnetic properties of the obtained sintered body of the present invention were determined. On the other hand, for comparison's sake, the same powdery alloy as raw material was sintered under the same conditions, and then the sintered body was subjected to aging at  $900^\circ C$  for 2 hours 40 and cooled to room temperature at a rate of  $200^\circ C/min$  in an argon atmosphere. This is the conventional method of producing rare earth-cobalt magnets. The magnetic properties of the sintered body were determined. Table 1 shows the comparison between both determinations.

Table 1

|                                                  | Br<br>(KG) | B <sup>HC</sup><br>(KOe) | I <sup>HC</sup><br>(KOe) | (BH) <sub>max</sub><br>(MG·Oe) |
|--------------------------------------------------|------------|--------------------------|--------------------------|--------------------------------|
| Magnet of<br>present invention                   | 8.20       | 8.00                     | 32.0                     | 16.8                           |
| Magnet Produced<br>by the Conventional<br>Method | 7.90       | 7.40                     | 24.0                     | 15.6                           |

In Table 1,  $B_r$  is residual magnetic flux density,  $B_{HC}$  normal coercive force found on B-H demagnetizing curve (B: magnetic flux density, H: intensity of magnetic field),  $I_{HC}$  intrinsic coercive force found on  $4\pi M$ -H demagnetizing curve ( $4\pi M$ : intensity of magnetization), and  $(BH)_{max}$  maximum energy product.

As seen in Table 1, the permanent magnet according to the present invention is excellent, compared with the magnet produced by the conventional method.

#### EXAMPLE 2

The same mixed powdery alloy as in example 1 was sintered under the same conditions, and then the obtained sintered body was cooled from sintering temperature to various quenching temperatures at a rate of  $6^{\circ}\text{C}/\text{min}$ . in a cooling rate controlled furnace. The sintered body thus cooled was immediately and quickly cooled successively from the quenching temperature to room temperature by blasting it with argon gas at the rate of about  $200^{\circ}\text{C}/\text{min}$ . FIG. 1 shows the influence of the quenching temperatures on the intrinsic coercive force  $I_{HC}$  of the obtained sintered body.

As seen in FIG. 1, the optimum quenching temperature is  $875^{\circ} \pm 50^{\circ}\text{C}$ .

#### EXAMPLE 3

Powdery alloy whose composition was Sm—40%Co was added to powdery alloy whose composition was Sm—66.2%Co to obtain mixed powdery alloy whose composition was Sm—63%Co. The resulting mixed powdery alloy was ground by a vibration mill for 4 hours to an average particle diameter of 3.3 m. The obtained fine powder was sintered by the same method and under the same conditions as that and those of the example 1. And then the sintered body was gradually cooled from the sintering temperature to quenching temperature of  $900^{\circ}\text{C}$  at a rate of  $0.8^{\circ}\text{C}/\text{min}$ . in a controlled furnace. The sintered body thus cooled was immediately and quickly cooled to room temperature. On the other hand, the same powdery alloy was sintered under the same conditions as mentioned above and cooled to the quenching temperature of  $900^{\circ}\text{C}$  at a rate of  $16^{\circ}\text{C}/\text{min}$ . When the sintered body was cooled to the quenching temperature of  $900^{\circ}\text{C}$ , it was immediately and quickly cooled to room temperature by blasting it with argon gas. Table 2 shows comparison between the magnetic properties of the magnet of the present invention and those of the magnets made by the conventional method.

Table 2

|                                            | $B_r$<br>(KG) | $B_{HC}$<br>(KOe) | $I_{HC}$<br>(KOe) | $(BH)_{max}$<br>(MG-Oe) |
|--------------------------------------------|---------------|-------------------|-------------------|-------------------------|
| Magnet of Present invention                | 8.40          | 8.18              | 28.0              | 17.8                    |
| Magnet Produced by the Conventional Method | 8.22          | 4.25              | 4.92              | 15.9                    |

As seen in Table 2, it is preferable to cool the sintered body gradually from the sintering temperature to the quenching temperature.

#### EXAMPLE 4

The same mixed powdery alloy as in the example 3 was sintered under the same conditions, and cooled

from the sintering temperature to the quenching temperature of  $900^{\circ}\text{C}$  at various cooling rates. When the sintered body was cooled to  $900^{\circ}\text{C}$ , it was immediately and quickly cooled to room temperature at a rate of  $200^{\circ}\text{C}/\text{min}$ . The graph in FIG. 2 shows the influence of the cooling rates from the sintering temperature to the quenching temperature on the intrinsic coercive force  $I_{HC}$  of the sintered body.

As seen in FIG. 2, the preferable cooling rate of the sintered body is slower than  $7^{\circ}\text{C}/\text{min}$ .

#### EXAMPLE 5

Powdery alloy whose composition was Sm—40%Co was added to powdery alloy whose composition was Pr—8.6% Sm—67.3%Co to obtain mixed powder alloy whose composition was Pr—16.7% Sm—63%Co. The resulting mixed powdery alloy was ground by a vibration mill for 70 min. to an average particle diameter of 3.2 m. The obtained fine powder was compressed to a green body by the same method as in example 1 and was sintered at  $1,130^{\circ}\text{C}$  for 1 hour. The sintered body was cooled from the sintering temperature to  $900^{\circ}\text{C}$  in a furnace at a rate of  $7^{\circ}\text{C}/\text{min}$ . After the sintered body was cooled to  $900^{\circ}\text{C}$ , it was immediately and quickly cooled to room temperature at a rate of  $200^{\circ}\text{C}/\text{min}$ . On the other hand, the same powdery alloy as raw material was sintered under the same conditions, and cooled in the furnace to  $700^{\circ}\text{C}$  at a rate of  $7^{\circ}\text{C}/\text{min}$ . When the sintered body was cooled to  $700^{\circ}\text{C}$ , it was immediately cooled to room temperature at a rate of  $200^{\circ}\text{C}/\text{min}$ . Table 3 shows comparisons between the magnetic properties of the magnet of the present invention and that produced by the conventional method.

Table 3

|                                            | $B_r$<br>(KG) | $B_{HC}$<br>(KOe) | $I_{HC}$<br>(KOe) | $(BH)_{max}$<br>(MG-Oe) |
|--------------------------------------------|---------------|-------------------|-------------------|-------------------------|
| Magnet of present invention                | 8.60          | 7.40              | 13.3              | 17.1                    |
| Magnet Produced by the Conventional Method | 8.60          | 6.82              | 10.2              | 16.16                   |

As seen in Table 3, the permanent magnet of the present invention has excellent magnetic properties, compared with the magnet produced by the conventional method.

#### EXAMPLE 6

Powdery alloy whose composition was Sm—66.2%Co and powdery alloy whose composition was Sm—40%Co were added to powder alloy whose composition was Pr—67.6%Co to obtain mixed powdery alloy whose composition was Pr—23.3% Sm—63%Co. The resulting mixed powder alloy was ground by a vibration mill for 25 minutes. The obtained fine powder was compressed to a green body by the same way as in the example 1. The green body was sintered at  $1,120^{\circ}\text{C}$  for 30 min, and gradually cooled to  $920^{\circ}\text{C}$  at a rate of  $6^{\circ}\text{C}/\text{min}$ . When the sintered body was cooled to  $920^{\circ}\text{C}$ , it was immediately and quickly cooled to room temperature. On the other hand, the same powdery alloy was sintered under the same conditions and immediately cooled to room temperature at a rate of  $250^{\circ}\text{C}/\text{min}$ . Table 4 shows comparison between the magnetic properties of the magnet of the present invention and those

of the magnet produced by the conventional method.

Table 4

|                                            | Br<br>(KG) | B <sup>HC</sup><br>(KOe) | I <sup>HC</sup><br>(KOe) | (BH) <sub>max</sub><br>(MG-Oe) |
|--------------------------------------------|------------|--------------------------|--------------------------|--------------------------------|
| Magnet of present invention                | 8.25       | 7.80                     | 12.5                     | 17.0                           |
| Magnet Produced by the Conventional Method | 7.80       | 5.80                     | 12.4                     | 13.1                           |

As seen in Table 4, the magnet of the present invention has excellent magnetic properties, compared with the magnet produced by the conventional method.

## EXAMPLE 7

Powdery alloy whose composition was Sm—40%Co was added to powdery alloy whose composition was Sm—66.2%Co to obtain mixed powdery alloy whose composition was Sm—63%Co. The resulting mixed powdery alloy was ground by a vibration mill for 4 hours to an average particle diameter of 3.3 m. The obtained fine powder was compressed to a green body by the same way as that of the example 1. The green body was sintered at 1,140°C for 1 hour, and gradually cooled to 900°C at a rate of 0.8°C/min. When the sintered body was cooled to 900°C, it was immediately cooled to room temperature at a rate of 100°C/min. by oil quenching. On the other hand, the same green body as mentioned above was sintered at 1,140°C for 1 hour and cooled to 900°C at a rate of 0.8°C/min. When the sintered body was cooled to 900°C, it was immediately cooled to room temperature at a rate of 4°C/min. by furnace cooling. Table 5 shows comparison between the magnetic properties of the magnet of the present invention and those of the magnet produced by the conventional method.

Table 5

|                                            | Br<br>(KG) | B <sup>HC</sup><br>(KOe) | I <sup>HC</sup><br>(KOe) | (BH) <sub>max</sub><br>(MG-Oe) |
|--------------------------------------------|------------|--------------------------|--------------------------|--------------------------------|
| Magnet of present invention                | 8.43       | 8.18                     | 28.5                     | 17.6                           |
| Magnet Produced by the Conventional Method | 8.25       | 5.41                     | 15.0                     | 16.0                           |

As seen in Table 5, the magnet which was cooled at faster cooling rate of the present invention has excellent magnetic properties, compared with the magnet produced by the conventional method.

## EXAMPLE 8

In the example 7, the influence of various cooling rates from 900°C on the intrinsic coercive force,  $H_C$  of the sintered body was studied. FIG. 3 shows the experimental results.

As seen in FIG. 3, the preferable cooling rate is 20°C/min. or faster.

## EXAMPLE 9

Alloy whose composition was Sm—63.8% was melted to obtain an ingot and the obtained ingot was preliminarily ground to prepare coarse powder.

The resulting coarse powdery alloy was ground by a vibration mill for 2½ hours to an average particle diam-

eter of 3.4 m. The obtained fine powder was compressed to a green body by the same way as that of the example 1. The green body was sintered at 1,110°C for 1 hour, and cooled to 830°C at a rate of 0.8°C/min. When the sintered body was cooled to 830°C, it was immediately cooled to room temperature at a rate of 200°C/min. On the other hand, the same powdery alloy was sintered under the same conditions and subjected to aging process at 900°C for 14 hours. Table 6 shows comparison between the magnetic properties of the magnet of the present invention and those of magnet produced by the conventional method.

Table 6

|                                            | Br<br>(KG) | B <sup>HC</sup><br>(KOe) | I <sup>HC</sup><br>(KOe) | (BH) <sub>max</sub><br>(MG-Oe) |
|--------------------------------------------|------------|--------------------------|--------------------------|--------------------------------|
| Magnet of present invention                | 8.00       | 8.00                     | 30.0                     | 16.0                           |
| Magnet Produced by the Conventional Method | 7.80       | 7.70                     | 12.0                     | 15.2                           |

As seen in Table 6, the magnet of the present invention has excellent magnetic properties.

## EXAMPLE 10

Alloy whose composition was Sm—63.8%Co was melted to obtain an ingot and the obtained ingot was ground to coarse powder. The resulting coarse powder was ground by a vibration mill for 3 hours. The obtained fine powder was compressed to a green body in magnetic field by the same way as in example 1. The green body was sintered at 1,130°C for 1 hour in an inert atmosphere, and gradually cooled for 850°C at a rate of 0.1°C/min. When the sintered body was cooled to 850°C, it was immediately cooled at a rate of 1,000°C/min. by blasting it with liquid carbonic acid gas. The magnetic properties of the sintered body was as follows:

$$\begin{aligned} Br &= 8.60 \text{ KG} \\ B^{HC} &= 8.60 \text{ KOe} \\ I^{HC} &= 34.0 \text{ KOe} \\ (BH)_{max} &= 20.1 \text{ MG.Oe} \end{aligned}$$

## EXAMPLE 11

Alloy whose composition was Sm—63.8%Co was melted to obtain an ingot, and the obtained ingot was ground to coarse powder. The resulting coarse powder was ground by a vibration mill for 3 hours. The obtained fine powder was compressed to a green body in magnetic field by the same way as in example 1. The green body was sintered at 1,170°C for 1 hour in an inert gas atmosphere, and gradually cooled to 850°C at a rate of 0.05°C/min. When the sintered body was cooled to 850°C, it was immediately cooled to room temperature. Table 7 shows the magnetic properties of the magnet obtained by this method.

Table 7

|    | Cooling rate<br>(°C/min) | I <sup>HC</sup><br>(KOe) | (BH) <sub>max</sub><br>(MG-Oe) |
|----|--------------------------|--------------------------|--------------------------------|
| 65 | 100                      | 27                       | 18.8                           |
|    | 400                      | 30                       | 20.0                           |
|    | 600                      | 35                       | 20.9                           |
|    | 1000                     | 37                       | 22.0                           |

The reason why quenching was performed at the temperature in the range of  $875^{\circ} \pm 50^{\circ}\text{C}$  in the present invention is that coercive force is decreased when quenching is conducted at temperatures not included in the above mentioned temperature range. The highest coercive force can be obtained when quenching is performed at the temperatures of  $850^{\circ}$  to  $900^{\circ}\text{C}$ .

On the other hand, the reason why the cooling from the sintering temperature to the quenching temperature is done at a rate of  $7^{\circ}\text{C}/\text{min}$  or slower rate is that when the cooling rate is faster than the above rate, coercive force is decreased remarkably. When the cooling rate is  $2^{\circ}\text{C}/\text{min}$  or slower, the best results can be obtained.

The reason why the cooling is performed at a rate of  $20^{\circ}\text{C}/\text{min}$  or faster rate in the quenching process is that if cooling is performed at a slower rate, coercive force is decreased. When cooling is performed at a rate of  $100^{\circ}\text{C}/\text{min}$  or faster in the quenching process, the highest coercive force can be obtained.

As mentioned above in detail, the present invention is characterized in that a green body having given composition is sintered, and gradually cooled from the sintering temperature to a given quenching temperature, and then quickly cooled to room temperature, without requiring after heat treatment.

The magnet according to the present invention has excellent coercive force as well as excellent residual magnetic flux density and energy product.

What is claimed is:

1. A method of producing a permanent magnet having a residual magnetic flux density of at least 8000 Gauss, a normal coercive force of at least 8000 Oersted, an intrinsic coercive force of at least 27,000 Oersted and a maximum energy product of at least  $17.6 \times 10^6$  Gauss Oersted comprising the steps of:

1. preparing a powdery alloy from about 55-70% by weight of cobalt and about 30-45% by weight of at least one rare earth element, selected from the

group consisting of Y, La, Ce, Pr, Sm, Nd, Gd, Ho and Er,

2. compacting said powdery alloy in a magnetic field,

3. sintering said compact at a temperature between

$1,000^{\circ}$  to  $1,200^{\circ}\text{C}$ .

4. cooling said sintered body from said sintering temperature to a quenching temperature in the range of about  $825^{\circ}$  to  $925^{\circ}\text{C}$ . at a rate no greater than  $7^{\circ}\text{C}/\text{min}$ , and

5. cooling said sintered body immediately from said quenching temperature to room temperature at a rate of at least  $20^{\circ}\text{C}/\text{min}$ .

2. A method of producing a permanent magnet according to claim 1, wherein said sintered body is cooled from the sintering temperature to the quenching temperature at a rate no greater than  $2^{\circ}\text{C}/\text{min}$  and further cooled immediately from the quenching temperature to room temperature at a rate of at least  $100^{\circ}\text{C}/\text{min}$ .

3. A method of producing a permanent magnet according to claim 1, wherein said sintered body is cooled from the sintering temperature to the quenching temperature at a rate no greater than  $0.1^{\circ}\text{C}/\text{min}$ . and further cooled immediately from the quenching temperature to room temperature at a rate of at least  $400^{\circ}\text{C}/\text{min}$ .

4. A method of producing a permanent magnet according to claim 3, wherein samarium-cobalt powdery alloy is used as the powdery alloy.

5. A method of producing a permanent magnet according to claim 3, wherein samarium-praseodymium-cobalt powdery alloy is used as the powdery alloy.

6. A method of producing a permanent magnet according to claim 1, wherein said sintered body is cooled from the sintering temperature to a quenching temperature of between  $850^{\circ}$  to  $900^{\circ}\text{C}$  at a rate no greater than  $0.1^{\circ}\text{C}/\text{min}$ , and the body thus cooled is further cooled immediately from the quenching temperature to room temperature at a rate of  $400^{\circ}\text{C}/\text{min}$ . or faster rate.

\* \* \* \* \*